

March 13, 1945.

A. R. ROWE

2,371,356

METHOD OF PRODUCING STEEL BILLETS

Filed July 20, 1943

Fig. 1.



WITNESSES.  
E. J. Maloney.

BY

INVENTOR.  
Andrew Reed Rowe  
Brown, Cuttler & Flick

ATTORNEYS.



## UNITED STATES PATENT OFFICE

2,371,356

## METHOD OF PRODUCING STEEL BILLETS

Andrew Reed Rowe, McKeesport, Pa., assignor to  
 National Tube Company, Pittsburgh, Pa., a  
 corporation of New Jersey

Application July 20, 1943, Serial No. 495,471

2 Claims. (Cl. 80—60)

The invention relates to the production of steel billets that are substantially rectangular in cross section, having rounded corners, and which are subsequently rolled or otherwise worked to form various sections, seamless tubing, forgings and the like.

The prevailing practice in producing such billets is to roll ingots into blooms on a reversing blooming mill which may be a two-high or a four-high mill whose working rolls are supported by backing rolls, and then on the same heat to roll the blooms singly on a reversing three-high mill or on a continuous mill which is used primarily for producing the smaller size billets. The working rolls of such billet mills are provided with grooved passes that are formed between deep collars that not infrequently spall and break, making it necessary to regrind the rolls or substitute new ones.

Before being rolled or otherwise worked, it is necessary to condition the four rolled surfaces of each such singly rolled billet, as by chipping, grinding, flame cutting or scarfing, which requires a substantial amount of time, and not infrequently is attended by a substantial loss of metal required to be removed.

The object of the invention is to provide an improved method of producing steel billets of the type explained, whereby the direct cost of production is materially reduced and substantial indirect savings are attained by reduction in the wear and breakage of rolls and roll collars.

In the practice of my improved method steel billets are produced in multiple from an ingot which is first rolled on a slabbing mill to form a slab having a thickness which is substantially equal to the thickness of desired billets and having a width which is a multiple of that of desired billets. Any well known or desired procedure may be followed to roll such slabs from cast ingots. They may be rolled on either two or four-high reversing slabbing mills having vertical edging rolls in line with horizontal slabbing rolls, but preferably the slabbing rolls are provided with one or more edging passes and the working tables adjacent to them are equipped to turn the slabs on their edges and properly guide them through the passes.

After a slab of the desired width and thickness has thus been produced it is, on the same heat, flat rolled in a closed pass to form desired rounded corners at its longitudinal edges, and also simultaneously to form narrow shallow grooves on the upper and lower faces of the slab, the grooves on the upper being opposed to those on the lower

face. These grooves have rounded corners and they are spaced from each other and from the edges of the slab the width of desired billets. While this grooving and corner-rounding pass 5 may be formed in the rolls of a special mill stand, it is preferably formed in the working rolls of the slabbing mill.

When the thus grooved slab has been formed it is flame cut in the plane of the opposed grooves 10 to form a plurality of billets, the flame cutting being done by oxyacetylene or oxyhydrogen torches which simultaneously finish the flame cut faces of the billets and make it unnecessary subsequently to condition them.

15 The invention will be further explained with reference to the accompanying drawing in which Fig. 1 is an elevation of the adjacent portions of a pair of slabbing rolls whose faces are also provided with edging passes and with a closed pass 20 finally to form opposed grooves in the faces of slabs; Figs. 2, 3, 4, 5, and 6 end views of a blank as it is rolled successively in the several passes of the rolls shown in Fig. 1; and Fig. 7 a perspective view of a grooved slab being flame cut to 25 produce a plurality of billets.

As shown in Fig. 1, the faces of upper slabbing roll 10 and lower slabbing roll 11 are provided with a slabbing pass 1, a preliminary edging pass 2, a final edging pass 3 and a closed slab-grooving 30 and corner-rounding pass 4. Upper roll 1 is shown in its lowermost position, and is adapted to be elevated in any desired manner by roll balances which urge it against screw-downs which are turned to the required vertical position to form 35 any desired pass spread. An ingot is reduced to a slab by giving it the required number of passes in slabbing pass 1 and edging pass 2. When thus reduced it is given a final edging pass or passes in edging and corner-rounding pass 3, and 40 is thereafter rolled in closed pass 4 to provide its upper and lower faces with narrow shallow grooves opposing each other, and also to form desired rounded corners on the longitudinal edges of the slab.

45 As shown in Fig. 1, pass 4 is shaped to provide two grooves in the upper and two in the lower face of a slab, the grooves being formed by small collars 7 on the faces of rolls 10 and 11. The outer portion 8 of each of these collars is curved 50 to correspondingly form a rounded base at the bottom of each groove, and, between the outer portions of each collar and the adjoining cylindrical roll faces, each roll is curved as at 9 to form rounded corners at the outer portions of the 55 grooves. The edges of pass 4 are formed by col-

lars 15 which are curved as at 16 to form rounded corners at the longitudinal edges of a grooved slab. The curvatures 16 of pass 4 may be of slightly less radius than the corresponding curvatures 18 in final edging pass 3 to provide an initial underfill at the corners of pass 4. In rolling a slab in pass 4 these corner underfills are filled by the displacement of metal incident to the forming of grooves by collar 7. Thus in pass 4 there is no overfill, and consequent formation of fins, in the plane of the meeting faces of the rolls at the edges of the pass.

Pass 4 may be formed to provide any desired number of properly spaced grooves in the upper and lower faces of a slab so that the slab may later be flame cut into any desired number of billets of a given size. By way of example, and not of limitation, the details of a suitable procedure will be explained for rolling slabs in multiples of three billets that are  $4\frac{1}{2} \times 4\frac{1}{2}$  inches in cross section. Starting with a steel ingot about  $23\frac{1}{2} \times 26\frac{1}{2}$  inches and weighing about 12,500 pounds, it is first given about ten passes in slabbing pass 1 to reduce it to a slab about  $20 \times 11$  inches, as shown in Fig. 2. The slab is then turned on its edge and is given four edging passes in edging pass 2 to reduce it to about  $15 \times 12$  inches, as shown in Fig. 3. The thus edged blank is then given four passes in slabbing pass 1 to reduce it to about  $19 \times 5$  inches, as shown in Fig. 4, and is then turned on its edge and given one or two edging passes in final edging and corner-rounding pass 3 to shape it to the form shown in Fig. 5 which is about  $14 \times 4\frac{1}{2}$  inches. The slab is finally given one or more passes in closed groove-forming pass 4 to provide its upper and lower faces with opposed narrow shallow grooves 20. These grooves may suitably be about three-sixteenths of an inch wide at their bases and one-half inch in depth. After the slab is thus rolled and grooved it is flame cut by torches 21 which burn slits through the slab of about three-sixteenths of an inch in width and leave the corners of the billets rounded to the same curvature as the rounded edges of groove 20.

In the example given the tonnage rate of production of grooved slabs of the form shown in Figs. 6 and 7 is three times greater than that of rolling billets singly according to the prevailing practice explained above. In other words, thirty tons of slabs of the form shown in Figs. 6 and 7 can be rolled in the time required for rolling ten tons of billets singly. Thus the rolling time per ton is greatly reduced, with a corresponding saving in the cost of billet production. Flame cutting of the slab into billets proceeds rapidly at the rate of about twenty-four inches

per minute, and the flame cut faces of the billets require no time-consuming conditioning, such as would be necessary if those faces had been rolled in forming the billets by conventional practice. The overall cost of flame cutting grooved slabs and conditioning their rolled faces is not more than that of conditioning all four faces of billets rolled singly according to the prevailing practice, and is usually less with an attendant saving in cost of billet production. In addition to these direct savings in the cost of billet production, there is less spalling and breakage of the shallow groove-forming collar 7 and of the working rolls than in the case of rolls which are provided with deep collars for rolling all four faces of billets singly. This indirect reduction in cost of producing billets is substantial.

According to the provisions of the patent statutes, I have explained the principle and mode of operation of my invention, have illustrated the preferred way of practicing it, and have given a specific example of one procedure. However, I desire to have it understood that, within the scope of the appended claims the invention may be practiced otherwise than specifically illustrated and described.

I claim:

1. The method of producing steel billets in multiple from an ingot, comprising rolling an ingot to form a slab having a thickness which is substantially equal to and a width which is a multiple of that of desired billets, rolling the slab in a closed pass to form rounded corners at its longitudinal edges and narrow shallow opposed grooves in the upper and lower faces thereof, such grooves having rounded corners and being spaced from each other and from the edges of the slab the width of desired billets, and flame cutting the slab in the planes of said opposed grooves to form a plurality of billets and simultaneously to finish the so cut faces of the billets.

2. The method of producing steel billets from an ingot, comprising rolling an ingot on a slabbing mill to form a slab having a thickness which is substantially equal to and a width which is a multiple of that of desired billets, rolling the slab in a closed pass provided in the rolls of said slabbing mill to form rounded corners at the longitudinal edges of the slab and opposed grooves in the upper and lower faces thereof, such grooves having rounded corners and being spaced from each other and from the edges of the slab the width of desired billets, and flame cutting the slab in the planes of said opposed grooves to form a plurality of billets and simultaneously to finish the so cut faces of the billets.

ANDREW REED ROWE.